

J. J. BYERS.

SHEET MATERIAL AND METHOD OF TREATING THE SAME.  
APPLICATION FILED JAN. 10, 1917.

1,325,075.

Patented Dec. 16, 1919.



Inventor:  
Joseph J. Byers,  
by Emery Booty, James W. Nance,  
Attys.

# UNITED STATES PATENT OFFICE.

JOSEPH J. BYERS, OF BROOKLINE, MASSACHUSETTS, ASSIGNOR TO PRODUCTS SYNDICATE, INC., OF BOSTON, MASSACHUSETTS, A CORPORATION OF MASSACHUSETTS.

## SHEET MATERIAL AND METHOD OF TREATING THE SAME.

1,325,075.

Specification of Letters Patent. Patented Dec. 16, 1919.

Application filed January 10, 1917. Serial No. 141,687.

To all whom it may concern:

Be it known that I, JOSEPH J. BYERS, a citizen of the United States, and a resident of Brookline, county of Norfolk, State of Massachusetts, have invented Improvements in Sheet Materials and Methods of Treating the Same, of which the following description, in connection with the accompanying drawings, is a specification, like characters on the drawings representing like parts.

This invention relates to the art of applying a sheet or layer of material to another, for the purpose of imparting thereto certain desirable qualities, as well as to the improved product obtained by said method. The invention is applicable to any sheet material, but the invention contemplates more particularly the application thereof to textile or other fibrous materials, such as leather for example, at least one of the sheets having preferably been treated so as to impart thereto wear-resisting and other advantageous qualities.

The invention will best be understood from the following description, taken in connection with the accompanying drawing, of one illustrative product of my improved method, and of the best mode or manner known to me for practising such method, 30 while its scope will be more particularly pointed out in the appended claims.

The accompanying drawing shows one improved product embodying my invention.

Referring to the drawing, the sheet of material 1 therein illustrated is given merely as an example of any textile or other fibrous material, such as leather for example, to which it is desired to apply another wear-receiving sheet 2.

The outer or wear-receiving sheet will preferably be treated to render the same water-repellent and highly wear-resisting, and is then so applied to the other sheet 1 as to constitute a homogeneous, wear-resisting layer.

Any suitable material may be taken as a basis for the wear-receiving sheet 2, but preferably this will be of some fibrous material such as a textile fabric or leather.

Certain materials, such as ordinary grades of chrome-tanned leather for example, which, owing to their porosity, lack of body and tendency to stretch when moist are not adapted for certain uses where wear-resisting or other special qualities are re-

quired, will, when treated by my process, become suitable for such uses.

The sheet material 2 which is to constitute the wear-receiving sheet or member is preferably treated with a cement-like substance 60 consisting of or including a cellulose derivative in solution and containing a quantity of non-oxidizing oil. This treatment is carried out in such a manner as to impregnate the material throughout with the oil-containing cement. This cement-like substance, containing a cellulose derivative and a non-oxidizing oil, will hereinafter be referred to briefly as the cement.

The materials composing the cement and the proportions in which they are mixed may be varied within wide limits. A suitable cement, for example, may be prepared by dissolving some cellulose derivative, a soluble nitrocellulose for example, in a suitable solvent, which may be acetone and alcohol in equal parts; if, for illustration, soluble nitro-cellulose and acetone and alcohol are used, one pound of soluble nitro-cellulose to one gallon of solvent may be employed with good results. To this is added a substantial amount of some non-oxidizing or non-drying oil, preferably a vegetable oil. This, for example, may be castor oil in the proportion of eight ounces to one pound of soluble nitro-cellulose.

The preferred method of impregnation is by immersing the material in a bath composed of the cement. For illustration, a bath may be prepared of sufficient volume 90 and proportion to the mass of the material to be treated to maintain the material immersed for the required time thoroughly to impregnate it without impairing the fluidity of the bath or effectiveness of the treatment. 95 The tank or other receptacle employed for the bath is closed to prevent any substantial evaporation of the solvent during the treatment of the material and is also provided with suitably controlled heating means so as to maintain the bath at a suitable temperature.

The temperature of the bath is preferably maintained at a point above the normal temperature of the air but below that which 105 would rapidly evaporate the solvent or impair the material to be treated. In the treatment of leather with a cement constituted as described and containing the stated amount of castor oil, the temperature should 110

be preferably less than 150° F. Good results are obtained with temperatures varying from 125° to 130° F.

Porous materials such as leather usually hold absorbed more or less hygroscopic moisture. To facilitate the impregnation of the material with cement, it is preferable to remove substantially all water and hygroscopic moisture from the material before its treatment. This may be accomplished in any suitable or desirable manner, but, in the case of leather, a simple method is to expose the material to a suitable drying temperature for a period long enough to drive out the moisture. The time and temperature required will differ for different materials and for different masses of the same material. In the case of leather, for example, the leather may be hung or spread over night in a drying room or a drying oven at a temperature of from 120° to 150° F. In the case of some textile fabrics or thin sheet material, the material may be prepared for immersion by passing the same slowly through a drying room or drying apparatus.

Preferably also the material should be handled and the treatment carried out in a room where the air has a low humidity, so that in passing from the drying operation to the immersion, the material may have no opportunity to absorb or collect any substantial or detrimental amount of moisture.

By expelling substantially all the moisture in the leather or other material, and immersing it while in a dry state, the permeation or impregnation of the material is facilitated and it is possible to impregnate the entire mass with the cement.

With the material dried as described, it may be immediately plunged into the bath and there maintained immersed in the presence of heat for a long enough period thoroughly to impregnate it with the cement.

The period during which the immersion may be profitably continued will vary with the material and its thickness. For sole or similar leather, for example, several minutes to several hours may be required, according to thickness. In the case of some thin, permeable material, a few minutes will sometimes be sufficient. The immersion is continued for an appreciable period, sufficiently prolonged to impregnate the material throughout. In the presence of heat and immersed in the solution, the material becomes thoroughly impregnated with the cement.

The material treated by this method will be thoroughly impregnated throughout as distinguished from a mere surface coating or a coating which has a mere anchorage or impregnation of limited depth. Leather thus treated acquires the property of repelling water, has great durability and density and a high degree of flexibility.

Furthermore, the water-repellent properties and flexibility are long continuing, which I attribute to the fact that the oil which is sealed into the fibers or particles by the cement cannot be washed out by exposure to moisture. When ordinary leather becomes wet and is thereafter dried by exposure to heat, it loses its softness and flexibility, becomes dry and hard and cracks very readily. This is largely due to the fact that the oil, soap or grease contained in the leather has been in part washed out by the wetting of the leather and in part driven out by the subsequent application of heat for drying the leather. Leather treated by my present method and which has become damp can be readily dried by the application of heat without becoming hard or stiff and without losing its flexibility and water-repellent properties, which I also attribute to the fact that the oil is sealed into the individual fibers or particles by the cement and cannot be driven out by the heat used to dry the leather.

It will thus be seen that leather treated by my process appears to have an oil-flexed property which is substantially permanent, while the oil commingled with the cement throughout the body gives it a high degree of permanent flexibility and water-repellent property.

After removing the material from the bath, it is dried, the effect of this is apparently to unite the fibers or particles into a homogeneous mass, leaving the oil sealed in the particles or fibers and protected by the cement, which as I believe, incases them and binds them together throughout.

The impregnated sheet material need not necessarily be absolutely dry but the drying should be sufficient to set the cement at or near the surface, and it is then ready to be applied to other material, to serve, for example, as a wear-receiving member or layer in respect to the latter. This will preferably be by cementing it thereto. Where the material treated in accordance with my process is applied directly to another material, for example leather or other fibrous material which has not been so treated, that face of the latter to which my treated material is to be applied will preferably be roughened up, so as to open up the fibers and permit the penetration of the cement solution used to a sufficient depth to secure a firm anchorage.

As an illustrative method of applying a fibrous material, leather for example, treated by my above-described process, to material, either leather or other fibrous material not so treated, the following may serve: One surface of the untreated material having been roughened as above stated, the same is covered with a cement solution, and a similar solution is applied to one face of the cement-impregnated material. Pref-

erably both materials should be warm and dry before application of the cement and the operation should preferably be carried out in a dry atmosphere. The cement employed for this coating is preferably a cement which contains a cellulose derivative and oil, and may be of the same nature as the cement used for impregnating the cement-impregnated material. Preferably, 5 however, it will be heavier or more concentrated than that cement, such, for example, as might be obtained by using one half or less of the solvent contained in the cement used for impregnation. The coating thus 10 applied to the surfaces to be united serves to fill the surfaces and to lay the nap or surface fibers. This coating is not merely anchored to the surface of the impregnated material but appears to become dissolved into and 15 united with the homogeneous cemented mass of the material and becomes a part thereof. When the coating thus applied to the two surfaces to be united has dried, one of said 20 surfaces is given another coating of adhesive cement, preferably the same as that used for impregnation, and while this coating of cement is still fluid, these two surfaces are applied to each other and are subjected to a 25 suitable even pressure throughout, this pressure being preferably maintained until the 30 cement is set. It is sometimes preferable to apply the solvent used to dissolve the cement, in place of this last coat of adhesive cement, the solvent thus applied apparently 35 sufficing to render the previous coating of cement sufficiently soft and tacky, firmly to unite the layers. Heat applied in conjunction with pressure will conduce to the evaporation of the solvent and the setting of the 40 cement. When the cement is set, the pressure may be removed and the resultant product allowed thoroughly to dry, when the two materials will be found to be 45 permanently cemented to each other. The pressure may be applied in any suitable manner or any suitable means, as for example by 50 subjecting the two superposed layers to direct pressure between heated presser members, such as flat plates, or between presser 55 rolls. But the direct pressure between two flat plates in a stationary press, so constructed that the plates will exert a substantially uniform continued pressure simultaneously on all parts of the material, or a considerable area thereof, for a more or less 60 prolonged interval, or until the cement is set, will in general be found more satisfactory. The pressure as applied will preferably be yielding; it serves to condense and 65 compact the cement-impregnated fibers of the material.

Instead of uniting a cement-impregnated material with one not cement-impregnated, two cement-impregnated materials may be 70 united by following the same mode of pro-

cedure above described, excepting that in such case, neither of the surfaces to be united will be roughened before applying thereto the preliminary cement coatings.

In all cases both materials to be united 70 will preferably be warm and dry before the adhesive coat of cement for uniting them is applied, and as already stated the operation will preferably be carried out in a dry atmosphere.

It will be apparent that any number of pieces or sheets of material may be united as described, all of said pieces or sheets being cement-impregnated or one or more being cement-impregnated sheets or pieces, 80 and one or more not. It will also be apparent that the alternative arrangement of the sheets or layers of material may vary as best suited to the purpose for which the resultant product is to be used, the cement-impregnated pieces or sheets and those not impregnated alternating either regularly or irregularly. Thus, where more than two pieces or sheets or layers of material are united, one or more that are not cement-impregnated may be embraced between two or more cement-impregnated ones, or vice versa, or two or more nonimpregnated pieces or sheets or layers may be provided with a single outer impregnated piece, layer 85 or sheet as a wear-receiving member, for 90 example.

It will also be apparent that where more than two layers of pieces of material are united in accordance with my process, they 100 may be united singly, or simultaneously in any numbers desired, it being borne in mind that where an impregnated piece is united to one that is not impregnated, as also where two unimpregnated pieces are united directly, the surface or surfaces of the unimpregnated piece or pieces to which the layer of cement is applied should preferably first be roughened.

The cement layer 3 by which the cement-impregnated pieces or sheets of material are 110 united appears to unite with the cement which permeates said pieces or sheets and forms therewith a homogeneous body. In the same manner the cement that unites a 115 cement-impregnated piece or sheet of material to one that is not so impregnated appears to unite so intimately with the fibers of the non-impregnated piece or sheet as well as with the cement which permeates 120 the cement-impregnated piece or sheet as to form with both of these a homogeneous body. The adhesive layer of cement also acquires the same flexibility and water-repellent characteristics as the impregnated 125 sheet material, so that it becomes one with the material that it unites, with no opportunity or tendency for separation thereat or therefrom, and such layer bends and flexes freely in unison with the pieces or sheets of 130

material that it unites, so that there appears to be an absence of wear-producing friction between said pieces. The pieces of material and the cement by which they are united and permeated appear to become one homogeneous mass that flexes as a single piece. The adhesive layer between the pieces or sheets renders the resultant product waterproof.

- 10 Certain fibrous materials, such as certain kinds of leather, chrome-tanned or other upper leather, for example, which lack resiliency and have a tendency to stretch, become unstretchable and gain resiliency 15 when treated by my process, which is a distinct advantage in the case of many uses to which my product may be applied. It will thus be seen that by my process, greater durability, toughness, compactness may be 20 imparted to leather or similar fibrous materials, than that possessed thereby before treatment. Furthermore, the leather or other fibrous material produced by this process is cement and oil-impregnated and 25 characterized throughout by a fibrous, cellular structure, the size and number of the air cells depending in part on the extent to which the condensing process has been carried out, the process thus rendering the 30 material substantially and permanently water-repellent, while imparting thereto some degree of porosity, so that it possesses an advantage over material of other non-porous, water-repellent or water-proof substances, such for example as rubber. Apparently the fibers become incased with the 35 cement after the material has been immersed, without necessarily wholly filling the interstices between the fibers or wholly 40 expelling the air from within the same.

It will thus be seen that by my process, durability, toughness, compactness and water-repellent qualities may be imparted to cheap or inferior grades of leather so as 45 to make them available for uses and purposes not heretofore possible, and as equal or better substitutes for leather of more expensive grades. Thus, in the case of chrome-tanned leather for example, the normally 50 porous and relatively loose structure of the leather becomes so charged with the cement that the leather has its fibrous structure compacted into a homogeneous, cement-bound, fibrous body. The cement adds to 55 the initial strength of the union of the fibers, but because of the oil still leaves the product flexible. The cement also adds its strength to the strength of the fibers, producing a homogeneous, compacted body 60 which can be worked in substantially the same manner as ordinary vegetable-tanned sole leather.

Leather treated by my process will buff and burnish to the same high degree as any 65 other leather and will take quite as perfect

a finish, upon its surfaces or edges, when treated by any usual burnishing or finishing process, and will retain that finish.

It will be understood that the terms "sheet" and "sheet material" used in the specification and claims, are used in their broad and comprehensive sense, as including for example any material such as leather, felt, or any textile, woven, or other permeable material in the web or piece. 75

It has been found that in some cases it is preferable to subject the leather to a degreasing process, in order to remove therefrom any excessive or undesirable oil or grease, or soap, before treating the leather 80 by my process. Any usual or well-known degreasing process may be employed for this purpose, such for example as immersing the leather for the required length of time in a bath of naphtha or benzin or other suitable 85 agent. In the case of textile fabrics the best results are obtained with unsized materials.

While I have herein described one illustrative example of my improved product and the several steps by which one form of 90 my product may be carried out, it is to be understood that my invention is not limited to the exact details specified or any of them, but that these may be varied within wide 95 limits without exceeding the true scope of my invention which is definitely set forth by the claims.

Having described my invention, what I claim as new and desire to secure by Letters Patent is:

1. The method of applying a sheet of leather or other permeable or fibrous material to another sheet of material, which is characterized by drying said sheets; impregnating one throughout with a cement containing a cellulose derivative and a non-oxidizing oil, by immersing it in a heated bath containing said cement in solution; applying to the surfaces of said sheets, by which they are to be united, a coating of cement also containing a cellulose derivative and a non-oxidizing oil; allowing said coatings to dry; applying to one of said surfaces a coating of adhesive cement; superimposing said surfaces while this coating of cement is still tacky; and compacting and cementing said sheets together by the application of pressure. 105

2. The method of applying a sheet of leather or other permeable or fibrous material to another which is characterized by drying said sheets; impregnating them throughout with a cement comprising a cellulose derivative and a non-oxidizing oil, by immersing them in a heated bath containing said cement in solution; applying to one surface of said sheets a coating of cement also containing a cellulose derivative and a non-oxidizing oil; allowing said coatings to dry; applying to one of said 110

cement-coated surfaces a coat of adhesive cement; superimposing said surfaces while this coating is still tacky; and compacting and cementing said sheets together by the application of pressure.

- 5 3. The method of applying a sheet of leather or other permeable or fibrous material to another sheet of material, which is characterized by degreasing the sheet to be applied; drying said sheets; impregnating one throughout with a cement containing a cellulose derivative and a non-oxidizing oil, by immersing it in a heated bath containing said cement in solution; applying 10 to the surfaces of said sheets, by which they are to be united, a coating of cement also containing a cellulose derivative and a non-oxidizing oil; allowing said coatings to dry; applying to one of said surfaces a coating 15 of adhesive cement; superimposing said surfaces while this coating of cement is still tacky; and compacting and cementing said sheets together by the application of pressure.
- 20 25 4. As a new article of manufacture a sheet of leather or other material having applied thereto a water-repellent, wear-resisting member, comprising a sheet or layer of leather or other fibrous or permeable

material, impregnating throughout with a 30 cement containing a cellulose derivative and a non-oxidizing oil and cemented to the first-named sheet by an adhesive cement.

5. As a new article of manufacture a sheet of leather or other material having 35 applied thereto a water-repellent, wear-resisting member, comprising a sheet or layer of leather or other permeable or fibrous material, impregnated throughout with a cement containing a cellulose derivative and 40 a non-oxidizing oil, and having its fibrous structure compacted into a cement-bound flexible body and being cemented to said first-named sheet by an adhesive cement.

6. As a new article of manufacture a 45 sheet of leather or other material having applied thereto a water-repellent, wear-resisting member, comprising a sheet or layer of leather or other fibrous or permeable material, impregnated throughout with a 50 cement containing a cellulose derivative and a non-oxidizing oil and cemented to the first-named sheet by an adhesive cement containing similar materials to that used to impregnate said sheet.

In testimony whereof I have signed my name to this specification.

JOSEPH J. BYERS.